

## UNITED STATES PATENT OFFICE

2,376,890

## CELLULOSE ESTER MANUFACTURE

Francis P. Alles, Waynesboro, Va., assignor to E. I.  
du Pont de Nemours & Company, Wilmington,  
Del., a corporation of Delaware

No Drawing. Application July 1, 1942,  
Serial No. 449,312

4 Claims. (Cl. 117—144)

This invention relates to the manufacture of cellulose organic ester structures having improved dyeing properties. More particularly it relates to the manufacture of wet coagulated cellulose organic ester structures which can be satisfactorily dyed with direct, acid and chrome dyes.

Generally speaking, cellulose organic ester structures have no affinity for direct dyes such as are commonly used for dyeing cotton and regenerated cellulose nor affinity for acid or chrome dyes such as are commonly used for dyeing silk and wool, unless they are chemically modified by suitable pretreatment. The only exception to this generalization is found in cellulose organic esters in a highly swollen state as may be produced by wet coagulation. Thus, "gel, wet-spun" cellulose acetate yarn, i. e., cellulose acetate yarn which has been made by the wet spinning process, and which is still in the freshly coagulated, undried state, accepts direct dyes, acid dyes, and chrome dyes. However, structures in the gel state are inherently weak and do not lend themselves conveniently to the usual textile operations such as twisting, winding, knitting, weaving or combing and carding, which precede dyeing. For this reason it has not been possible heretofore to take advantage of the superior dyeing properties of this material in commercial practice.

An object of this invention, therefore, is to preserve in dry wet-coagulated cellulose organic ester structures, the dyeing properties which characterize such structures in the gel or wet, freshly coagulated state.

Another object is to maintain the characteristic dye affinity of gel, wet-spun cellulose organic ester yarn through the drying step, whereby, on rewetting, the yarn may be dyed with acid, direct, and chrome dyes.

A still further object is to treat wet-spun cellulose acetate yarn in the gel state in order to maintain its affinity for acid, direct, and chrome dyes through the drying step.

These and other objects will more clearly appear hereinafter.

These objects are realized by my invention which, briefly stated, comprises impregnating gel, wet-coagulated cellulose organic ester structures with a solution of a bulk agent.

By the term "bulk" agent is meant any relatively non-volatile impregnant which can fill the capillaries or spaces between molecules or crystallites of the cellulose ester and prevent substantial collapse of these cell walls on drying.

Preferred bulk agents are polyhydric alcohols such as glycerin, sugar, corn syrup, and the like.

Preferably, the gel, wet-coagulated cellulose organic ester structure is impregnated with a solution of a bulk agent of sufficient concentration to give 15 to 400 parts by weight of solid per 100 parts of cellulose ester.

The following examples further illustrate my invention. Percentage compositions are by weight unless otherwise indicated.

*Example I*

10 A solution consisting of 15% cellulose acetate (containing about 54.5% combined acetic acid), 5% water, and 80% acetic acid, was spun into a coagulating bath consisting of 12% acetic acid, 15 13.5% ammonium acetate, and 74.5% water, which coagulating bath was maintained at a temperature of 8.50 C. The filament bundle consisting of 240 filaments of 20 denier each was washed free of acetic acid and wet reeled into a number of 20 small skeins. A number of these skeins of gel 25 yarn were impregnated by immersion in an aqueous solution containing 4% by volume of glycerin and 27% by volume of commercial corn syrup sold by Corn Products Refining Company under the name of "Karo," after which the skeins were wrung so as to retain about 1 part of non-volatile material per part of cellulose acetate when air-dried.

30 (a) One of these skeins, after being air-dried, was dyed by direct immersion in a dye bath comprised of du Pont Pontamine Fast Green GL, a direct dyestuff, to a deep shade of green comparable to that obtained by a corresponding dyeing of viscose rayon. Wash, light, and fume-fastness were excellent.

35 (b) Another impregnated and dried skein was rinsed thoroughly to remove all the corn syrup and glycerin and then dyed while still wet by immersion in a dye bath of du Pont Brilliant Milling Green B Conc. (Color Index No. 667) to a depth comparable to that obtained by a corresponding dyeing of wool. Light-fastness and wash-fastness were excellent.

*Example II*

40 A skein of gel yarn produced in accordance with Example I was impregnated with an aqueous solution of 10% (by volume) of commercial corn syrup sold by Corn Products Refining Company under the name of "Two-Star" corn syrup of 42° Bé. and a purity of 61.5. The treated skein was wrung so as to retain about 1 part of corn syrup 45 solids per 3 parts of cellulose acetate after being dried at room temperature. This dried skein of 50 yarn when immersed in a dye bath of du Pont

Pontamine Fast Black L (Color Index No. 363) dyed to a deep black shade.

*Example III*

1.5 inch, 3 denier cellulose acetate staple produced from filament bundles spun substantially as described in Example I was thoroughly impregnated with an aqueous solution consisting of 28% "Karo" corn syrup and 5% glycerol. The impregnated staple was wrung so as to retain one part of nonvolatile impregnants per part of cellulose acetate after air drying at room temperature. A wad of the dried staple was rinsed in water, wrung and then entered into an aqueous dye bath of du Pont Pontachrome Black F (Color Index No. 299) and dyed according to the usual procedure. The depth of dyeing observed was equivalent to that obtained by a corresponding treatment of wool. Light-fastness and wash-fastness were excellent.

*Example IV*

A skein of gel, wet-spun cellulose acetate yarn such as described in Example I was impregnated with an aqueous solution of 15% Gardinol WA, (the sodium salt of the alcohol acid sulfate of a fraction of the alcohols obtained by hydrogenating coconut oil, mainly sodium lauryl sulfate), wrung out and air dried. The dried skein was thereafter rinsed in water to remove the Gardinol and dyed with Pontamine Fast Red 8BL (Color Index No. 278) to produce a depth of dyeing equal to that obtained in corresponding direct dyeing of viscose rayon. Light-fastness and wash-fastness were excellent.

*Example V*

A gel, wet-spun cellulose acetate yarn was impregnated with an aqueous solution containing 20% polyethylene oxide (1500 molecular weight) and wrung so as to retain about 1 part of polyethylene oxide per part of cellulose acetate and air dried. After rinsing in water to remove the polyethylene oxide, the yarn was dyed with Pontamine Fast Red 8BL (Color Index No. 278). Depth of dyeing was equivalent to that obtained by similarly dyeing viscose rayon.

*Example VI*

A skein of gel, wet-spun cellulose acetate yarn was impregnated with an 80% aqueous solution of glycerol, wrung and air dried. The dried yarn was subsequently thoroughly rinsed in water to remove the glycerol and then dyed with du Pont Pontamine Sky Blue 6BX (Color Index No. 518). The dyeing was equivalent to that of viscose rayon.

*Example VII*

A skein of gel, wet-spun cellulose acetate yarn was impregnated with an aqueous solution consisting of 5% by volume of commercial corn syrup such as used in Example II and 5% by weight of sodium chloride, wrung and air dried. The resulting dried yarn was thoroughly rinsed in water to remove the bulking agent and then dyed with du Pont Pontamine Fast Red 8BL (Color Index No. 278). Good dyeing was obtained.

It is to be understood, of course, that the above examples are merely for purposes of illustration and that my invention is not limited to the materials, agents and proportions therein recited but is susceptible rather to wide variation.

Thus, although this invention has been described in terms of treating gel, wet-spun cellulose acetate yarn of the acetone soluble variety

to improve its affinity for direct, acid and chrome dyes, the invention is also applicable to the treatment of other formed structures such as film, sheeting, tubes, bands, and the like. Other cellulose acetates, such as substantially completely acetylated cellulose acetate commonly termed cellulose triacetate, as well as other cellulose esters such as cellulose propionate, cellulose butyrate, mixed esters such as cellulose acetate butyrate, cellulose acetate propionate and the like, may be likewise treated with good results.

In addition to the bulking agents described above, examples of satisfactory bulk agents are molasses, dextrose, dextrose, maltose, sucrose, ethylene glycol, diethylene glycol, gelatin, casein, albumin, polymethacrylic acid, quebracho extract, gum arabic, urea, inorganic salts, and pectic acid salts. Any relatively non-volatile material that can be uniformly impregnated into the gel, wet-coagulated cellulose organic ester structure can be employed. Preferably these materials are water-soluble, for impregnation is most convenient from aqueous solutions, since the structure to be impregnated is already highly swollen with water. However, other liquids, which are solvents for the bulk agents but not solvents for the cellulose ester and possessing relatively high vapor pressures, may be used as the vehicle for the bulk agent. Corn syrup is especially effective

wet-coagulated cellulose organic ester structure as a bulk agent because it does not crystallize readily and, as water is removed from the impregnated structure, the syrup becomes increasingly more viscous until it is substantially a solid, but yet an amorphous high viscosity fluid.

Cellulose acetate yarn processed and dyed in accordance with this invention is unusually light-fast and wash-fast, in some cases even more light and wash-fast than cellulose dyed with the same direct dye. Very probably the high degree of fastness is due to the fact that the dye penetrates to the very center of the fibers or filaments, whereas the processes suggested heretofore to modify the dyeing of cellulose derivative threads rendered only the surface of the yarn capable of accepting dye and had been merely a surface dyeing effect. Naturally, this kind of dyeing is much more susceptible to fading, either through washing or due to the action of sunlight.

I claim:

1. In the process of manufacturing cellulose acetate structures wherein the structures are formed in a coagulating bath, the steps which comprise impregnating the structures while still in the freshly coagulated gel state with corn syrup, and thereafter drying said structures.

2. In the process of manufacturing cellulose acetate structures wherein the structures are formed in a coagulating bath, the steps which comprise impregnating the structures while still in the freshly coagulated gel state with corn syrup and glycerin, and thereafter drying said structures.

3. A dry cellulose acetate structure having substantially uncollapsed capillaries filled with corn syrup and extending throughout the entire cross sectional area of the structure, said structure being capable of accepting direct, acid and chrome dyes.

4. A dry cellulose acetate structure having substantially uncollapsed capillaries filled with corn syrup and glycerin and extending throughout the entire cross sectional area of the structure, said structure being capable of accepting direct, acid, and chrome dyes.